

## UNITED STATES PATENT OFFICE

HANS T. CLARKE AND CARL J. MALM, OF ROCHESTER, NEW YORK, ASSIGNEES TO EASTMAN KODAK COMPANY, OF ROCHESTER, NEW YORK, A CORPORATION OF NEW YORK

## PROCESS OF MAKING UNSATURATED ACYL CELLULOSE ESTERS

No Drawing.

Application filed May 4, 1927. Serial No. 188,861.

This invention relates to a simplified process of making cellulose esters containing unsaturated acyl groups. One object of our invention is to provide a relatively simple and inexpensive process of producing cellulose esters containing an acyl group corresponding to a monocarboxylic unsaturated organic acid in which there is an ethylenic bond. Another object of the invention is to provide such a process in which the introduction of an acyl group from a lower member of the acrylic acid series is introduced by a simple single step. Another object of the invention is to provide a process in which the introduction of the unsaturated acid to the ester is carried out first, and then other acyl groups of the ester may be subsequently introduced. Other objects will hereinafter appear.

We have found that cellulose esters containing small but useful amounts of unsaturated acyl groups may be prepared by simply heating cellulose, either native or in a slightly hydrated form, in a bath containing the unsaturated acid and a solvent which lowers the boiling point of the mixture below a temperature at which harmful degradation of the cellulose occurs. We have also found that these lower esters of cellulose containing unsaturated acyl groups, are very readily esterified further by the known methods of introducing saturated groups, such as those corresponding to the fatty acids. It will thus be seen that we have provided a very simple single-stage method of producing cellulose esters containing useful amounts of unsaturated acyl groups, and a relatively simple two-stage process in which such lower esters are first formed and then further esterification is carried out in the usual way. While native cellulose is esterified by heating with unsaturated acids as above indicated, the esterification is neither so rapid nor so extensive as is the case with hydrated cellulose, so that we prefer to carry out the first stage of our process with either reverted cellulose, such as is produced in the manufacture of rayon fibers by the viscose or cuprammonium methods,—or cellulose which has been mercerized and its surface left in a reactive condition, say by suitable dehydration. For con-

venience in this particular application, we shall refer to all such forms of cellulose as "partially hydrated."

We shall now describe several forms of our invention by way of illustration, but it will be understood that our invention is not restricted to the details thus given, except as indicated in the appended claims. 20 parts by weight of rayon fibers from the cuprammonium process are placed in a mixture of 300 parts by weight of crotonic acid and 50 parts by weight of chlorobenzene, and the mixture heated for 48 hours at 155 to 157° C. The presence of the chlorobenzene lowers the boiling point and gives a good liquid bath at these temperatures which are reasonably safe with respect to the cellulose and the esters which are formed therefrom. In general we preferably work at least below 170° C. Occasionally the moisture is removed by distilling off chlorobenzene and replacing it with the same amount of dry chlorobenzene. The fibers now consist, not of plain reverted cellulose, but of lower cellulose crotonate esters. Such fibers are useful by themselves in this condition, because the unsaturated acyl groups in them offer points at which chemical modifications or substitutions may be made, thus providing for special dyeing treatment, for example. They contain 4.8% by weight of crotonyl groups.

The lower crotonates described in the preceding paragraph may be further esterified in any of the usual ways. If an aceto-crotonate is to be produced, they may be added to a regular acetylating mixture, such as one containing 30 parts by weight of acetic acid, 20 parts by weight of acetic anhydrid, and 1 part by weight of fused or anhydrous zinc chlorid. Into this bath 5 parts by weight of the above described lower crotonates are stirred and the mixture warmed at 60 to 65° C. until a homogeneous dope is obtained. From this dope the cellulose aceto-crotonates are precipitated by means of water, and the product washed and dried. It is soluble in chloroform, or acetone, or mixtures of them and yields transparent colloidized films upon the drying of its solutions.

In another form of our invention long

55

60

65

70

75

80

85

90

95

100

fibered cotton is mercerized for 48 hours in an 18% sodium hydroxide solution, pressed out, washed free of alkali, and then freed from water by washing with alcohol and ether, finally being dried. The combination of the mercerizing action and the special dehydrating leaves the fibers with the surface in a specially good condition for further reaction. 20 parts by weight of the mercerized and dehydrated fibers are then heated in a boiling mixture of 500 parts by weight of crotonic acid and 100 parts by weight of chlorobenzene. The temperature remains at 155 to 157° C. Chlorobenzene is a good example of an inert liquid which lowers the boiling point to a degree where the temperature is safe for the reaction and the products. The water liberated by the reaction is periodically removed by distillation, the chlorobenzene which distills out being replaced with dry chlorobenzene. After 48 hours' treatment, there is approximately 4.9% by weight of crotonyl groups combined with the cellulose, and after 96 hours' treatment there is about 6.7% of crotonyl groups in the lower esters thus produced. Where native cellulose, such as clean cellulose fibers or paper as used in manufacturing cellulose acetate, is substituted for the mercerized cellulose in the above example, the amount of crotonic groups introduced by the boiling is about one-fourth the amount introduced into the mercerized cellulose for an equal time of treatment.

The resulting fibers are useful, by themselves, after washing and drying, because of the chemical operations which may be carried out with respect to them by reason of the double bond in the crotonic groups. But these esters are likewise well adapted for the production of higher cellulose esters, that is, esters in which there are more acyl groups. The additional acyl groups may be added by any well known acylating bath. For example, either the fibers which have been given the 48 hour boiling treatment above, or those which have had 96 hours of such treatment, may be acetylated. 5 parts by weight of such fibers are introduced into 15 parts by weight of acetic anhydrid, and 20 parts by weight of acetic acid, along with 0.1 part by weight of magnesium perchlorate. The reaction is conducted at 60 to 65° C., the end point being indicated by the mass becoming homogeneous. From this mass the aceto-crotonates are obtained by precipitation with water or methyl alcohol, and washed by means of the latter. The product is soluble in acetone or chloroform or mixtures of them and yields transparent films from the evaporation of its solutions.

Stearyl groups may be introduced into the lower crotonates hereinabove described, as follows: 4 parts by weight of the lower cellulose crotonate fibers are mixed into 30 parts by weight of commercial stearic acid, 50 parts

by weight of chloroacetic anhydrid, and 0.1 part by weight of magnesium perchlorate. The mixture is kept at 60 to 65° C. until a homogeneous solution or dope is obtained, say in about 20 hours. The resulting dope is poured into methyl alcohol, and the precipitated cellulose crotono-stearate (or stearo-crotonate) is washed with warm methyl alcohol and dried. It is soluble in chloroform and benzol, and yields flexible, transparent skins upon evaporation of its solutions.

Of the other members of the acrylic series of unsaturated acids undecylenic may be used along with a solvent which reduces its boiling point sufficiently, but in general, we prefer to use crotonic acid, because of its lower boiling point and greater activity. Cinnamic acid is likewise useful.

The lower esters containing unsaturated acyl groups introduced by our simplified heating step may be further esterified, not only with acetyl groups or stearyl groups, as explained in the above illustrations, but with any of the groups introduced by the methods disclosed in our copending application Serial No. 179,177, filed March 28th, 1927, for Process of making cellulose esters of organic acids. In said application cellulose esters are prepared by using one or more of the group of carboxylic acids contained in the sub-groups consisting of the unsubstituted aliphatic monocarboxylic acids including the cycloparaffinic, the aromatic monocarboxylic acids and the aralkyl monocarboxylic acids, typical members of these carboxylic groups being the following: acetic, propionic, n-butyric, iso-butyric, n-valeric, iso-valeric, n-caproic, n-heptylic, caprylic, pelargonic, capric, lauric, myristic, palmitic, stearic, crotonic, cyclohexane-carboxylic, benzoic, o-methoxy-benzoic, o-chloro-benzoic, acetyl-salicylic, phenylacetic, hydrocinnamic and cinnamic. The acid with which the cellulose is to be esterified is mixed with the cellulosic material and a catalyst in the presence of an organic acid anhydrid which impels the esterification and preferably does not itself furnish groups to the ester, the halogen substituted fatty acid anhydrids having less than 10 carbon atoms, such as chloracetic anhydrid, being especially emphasized.

Of course, should an unsubstituted aliphatic monocarboxylic acid in which there is an ethylenic bond, such as crotonic acid, be used for the first esterification step it would not be frequent that it would be desired to further esterify with the same acid or one of similar molecular construction, it being preferable to further esterify with one of the other acids mentioned.

Having thus described our invention, what we claim as new and desire to secure by Letters Patent is:

1. In the process of making organic esters of cellulose, heating together a cellulose and

70

75

80

90

95

100

105

110

115

120

125

130

- 5 a monocarboxylic organic acid in which there is an ethylenic bond until a lower cellulose ester containing an unsaturated acyl group is produced, the temperature of the ingredients being maintained below the degradation points of the cellulose and the ester.
- 10 2. In the process of making organic esters of cellulose, boiling partially hydrated cellulose in a bath containing a monocarboxylic organic acid in which there is an ethylenic bond and a liquid miscible with said acid which is inert toward the cellulose and produces with the acid a mixture boiling below the degradation point of the cellulose, said boiling being continued until a lower cellulose ester containing an unsaturated acyl group is produced.
- 15 3. In the process of making organic esters of cellulose, heating together partially hydrated cellulose and crotonic acid, until a lower cellulose crotonate is produced, the temperature of the ingredients being maintained below the degradation points of the cellulose and the cellulose crotonate.
- 20 4. In the process of making organic esters of cellulose, boiling partially hydrated cellulose in a bath containing crotonic acid and a solvent thereof which is inert toward the cellulose and produces with the acid a mixture boiling below the degradation point of the cellulose, said boiling being continued until a lower cellulose crotonate is produced.
- 25 5. In the process of making organic esters of cellulose, boiling mercerized cellulose in a bath containing crotonic acid and chlorobenzol, at a temperature between 155 and 160° C. for at least 48 hours, and thereafter separating the lower cellulose crotonate, thus formed, from the reaction mixture.
- 30 6. In the process of making organic esters of cellulose, heating together partially hydrated cellulose and a monocarboxylic organic acid in which there is an ethylenic bond until a lower cellulose ester containing an unsaturated acyl group is produced, and thereafter further esterifying said lower cellulose ester.
- 35 7. In the process of making organic esters of cellulose, boiling partially hydrated cellulose in a bath containing a monocarboxylic organic acid in which there is an ethylenic bond and a liquid miscible with said acid which is inert toward the cellulose and produces with the acid a mixture boiling below the boiling points of either said acid or said liquid, said boiling being continued until a lower cellulose ester containing an unsaturated acyl group is produced, and thereafter further esterifying said lower ester in an anhydrid bath containing reactive fatty acid groups.
- 40 8. In the process of making organic esters of cellulose, boiling partially hydrated cellulose in a bath containing crotonic acid and a liquid which is inert toward the cellulose and
- 45 produces with the acid a mixture boiling below the boiling point of the latter, said boiling being continued until a lower cellulose ester containing a crotonic group is produced, and thereafter further esterifying said lower ester. 70
- 50 9. In the process of making organic esters of cellulose, boiling mercerized and dehydrated cellulose in a bath of crotonic acid and chlorobenzol until a lower cellulose crotonate is produced, and thereafter further esterifying said lower crotonate in an esterifying bath containing acetic anhydrid. 75
- 55 Signed at Rochester, New York, this 29th day of April, 1927. 80
- HANS T. CLARKE.  
CARL J. MALM.